

Patented Dec. 15, 1925.

1,566,000

# UNITED STATES PATENT OFFICE.

RICHARD W. HANNA, OF PIEDMONT, AND ORVILLE ELLSWORTH CUSHMAN AND THEODORE WILLIAM DOELL, OF BERKELEY, CALIFORNIA, ASSIGNORS TO STAND-ARD OIL COMPANY, OF SAN FRANCISCO, CALIFORNIA, A CORPORATION OF CALIFORNIA.

## PROCESS OF MANUFACTURING LUBRICATING OILS.

No Drawing.

Application filed April 28, 1924. Serial No. 709,681.

To all whom it may concern:

Be it known that we, RICHARD W. HANNA, ORVILLE ELLSWORTH CUSHMAN, and THEODORE WILLIAM DOELL, citizens of the United States, and residing in the cities of Piedmont and Berkeley, respectively, county of Alameda, and State of California, have invented a new and useful Process of Manufacturing Lubricating Oils, of which the following is a specification.

This invention relates to the art of manufacturing lubricating oils from petroleum oils.

In the copending application of Richard W. Hanna, John B. Terry, Ralph A. Holloran and Edwin D. Gray, Serial No. 591,638, filed September 30, 1922, there is set forth a process of manufacturing improved and high grade lubricating oils wherein a petroleum oil is subjected to requisite conditions of pressure and temperature in order to decompose a part of such oil and to polymerize and stabilize the residuum. The residuum, from such polymerizing and stabilizing action is then utilized to produce a highly stabilized lubricating oil, all as more fully set forth in the application mentioned above.

As was also pointed out in this copending application the prior production of lubricating oils has proceeded under the common theory of the art that high temperature and prolonged heating in the treatment or distillation of petroleum had a detrimental and undesirable effect on the quality of the lubricating oil which would be produced. It has been generally considered that under heat and pressure lubricating stocks were cracked and rendered more unstable and that generally the oil was rendered inferior for lubricating purposes. In accordance with this theory the distillation of petroleum for the production of lubricating oil has been conducted under the minimum heating and lowest temperature which economical considerations would permit.

It was pointed out in the copending application heretofore referred to that while high temperature, prolonged heating, or destructive distillation decomposes a part of the lubricating stock, the body of the residual oil has undergone a very marked change and that there exist fractions in the

residual oil fully as high or higher in viscosity than the original oil, and that these fractions have been stabilized and greatly improved in a number of respects. It appears that under the requisite heating and pressure the unstable fractions of the petroleum oil are either cracked and distilled off, thus being removed from the residuum, or that they are polymerized and retained in the oil in a much more stable form than they existed previously to the heating or cracking process.

It was the practice as set forth in the above mentioned copending application, to distill the residuum so desired in order to separate the oil content thereof from the tar and carbonaceous matter which results from a decomposition of certain ingredients or unstable fractions of the petroleum oil which is so distilled for a lubricating oil stock. The separate fractions having the viscosity desired for the production of lubricating oil were then separated from the relatively less viscous fractions by a reducing operation. The reduced oil was then refined with an acid if desired and the acid-treated oil filtered or otherwise clarified.

The present invention is an improvement of process described in the copending application referred to above and discloses certain improvements in the method as therein set forth.

It sometimes becomes desirable to produce a lubricating oil which will possess a rich green fluorescence, that is, when viewed by reflected light will possess a green color. It is also known to those familiar with the art that oils without this green fluorescence are generally characterized by a bluish color when viewed by reflected light.

Various reasons have been given for the presence of this green fluorescence in certain oils and a blue color in others. It is generally true that an oil produced from an overhead stock, that is, a stock that has been subjected to distillation for its separation from a base, in which distillation certain desired fractions are thrown over, will have a blue fluorescence whereas an oil made from a stock not so distilled or a stock from a bottom will have a green fluorescence. Thus in the manufacture of lubricating oils from eastern or paraffine base oils a rich green

fluorescence will result if the residuum remaining, after the removal of the gasoline, kerosene and other light fractions, is not subjected to a distillation wherein cracking

5 temperatures are reached for the conversion of the wax into the crystalline state, so that the wax may be removed by a wax-pressing process; in other words, if the wax is removed from the residuum by a cold settling  
10 or by a centrifuging method or other method whereby the wax may be removed in the amorphous state without the production of an overhead stock by a distillation process, a rich green fluorescence will result. When  
15 such distillation is resorted to for the conversion of the wax into the crystalline state, a blue fluorescence results.

It will thus be seen that especially in the production of lubricating oils from asphaltic or mixed base crude wherein it is necessary to conduct a distilling operation to separate the lubricating oil as an overhead stock from the asphaltic residuum, the resulting oil as heretofore manufactured will 20 be characterized by a bluish fluorescence.

So far as we are able to ascertain there has not heretofore been known a satisfactory method for the production of a lubricating oil, from an asphaltic or mixed base 30 crude, having a rich green fluorescence; nor from an eastern or paraffine base oil, if during the manufacture of the lubricating oil, the wax is converted into the crystalline state by a distillation operation wherein the lubricating oil stock is thrown over as a distillate.

We have discovered a method whereby this may be satisfactorily and economically accomplished. At the same time we are able 40 to produce such an improved lubricating oil in a very much larger quantity from the same stock than has heretofore been possible. Our invention embodies the preparation of a highly stabilized lubricating oil stock possessing to a great degree the desired green fluorescence and then blending or mixing this fluorescent stock with a lubricating oil stock which has been prepared by standard methods. This latter stock to which the green fluorescent stock 45 is added may be either the finished lubricating oil or it may be the stock from which the finished oil is to be prepared by standard methods. Likewise the green fluorescent stock may be taken 50 through a complete refining process for the production of a finished oil before it is added, in which case it is customarily added to a finished oil which has been prepared by standard methods, or it may be added in 55 an untreated or unrefined state to the stock from which the lubricating oil which is prepared by standard methods is made, in which case the resulting mixture is treated by the normal or standard methods.

65 With the foregoing preliminary explana-

tion our invention will be readily understood from the following description of a preferred process embodying the principles of our invention:

We prefer to employ heavy fractions of 70 petroleum which normally are treated for the production of lubricating oils, either with or without lighter fractions or solvent oil. To obtain these heavy fractions we prefer to first distill the crude oil under reduced pressures, less than atmospheric. Distillation under vacuum serves to preserve the hydrogen content of the oil and has a marked beneficial action on the remainder of the process. The fractions are 75 then destructively distilled under pressure and high temperature and the residual oil used for the production of lubricating oil. Normally, the temperature in the destructive distilling operation is from 650° F. to 80 800° F., and the pressure from 50 to 150 pounds above atmospheric.

As an alternate method the petroleum oil may be subjected to requisite temperature and pressure to decompose or crack a part 90 of such oil while producing a residuum containing the desired stabilized lubricating oil stocks having the green bloom, in a digestion process, that is a process wherein the produced lower boiling point oils are 95 held under sufficient pressure to substantially prevent their vaporization during the decomposing and stabilizing reactions. In which case the produced low boiling point 100 oils may be separated from the petroleum oils not converted into low boiling point oils by a subsequent distillation or reducing operation.

When destructively distilling the oil the 105 temperature and pressure and the time of heating will vary with the oil to be treated and the degree of decomposition desired. With certain oils a temperature as low 650° F. and a pressure of 10 pounds above atmospheric will be sufficient. It will normally be found that the quality of finally produced lubricating oil can be controlled by controlling the degree of destructive distillation or heat treatment to which the oil 110 is subjected under the proper conditions of 115 temperature and pressure. The greater the degree of cracking the more stable will be resulting lubricating oil.

We have found that the resulting yield 120 and quality of the lubricating oil obtained from the residual oil of a cracking process is influenced by the degree to which destructive distillation is carried. Also that for various stocks destructively treated, various degrees of cracking must be effected to produce the best results in the production of the lubricating stocks. As an illustration:

For a cracking stock composed of fractions which may be normally considered as 125 lubricating fractions, the yield and quality 130

of the finished lubricating oils from this process decreases after 20% of the original stock has been cracked and distilled over. On the other hand, when the heavy charging stock is mixed with say 40% of a lighter or solvent oil and destructively distilled, there is no decrease in yield or quality until after about 35% of the original charge has been cracked and distilled off.

10 During this destructive distillation it will be found that a large amount of the bodies that are unstable under the conditions of temperature and pressure employed have been cracked and distilled from

15 the residual, or such unstable constituents have been polymerized and retained in the residual in a form more stable at this temperature and pressure than the original oil.

Thus far our process is the same as that 20 set forth in the copending application referred to above. From this point on we combine therewith the improvements embodied in our present invention.

The residuum obtained by the process as 25 set forth above is preferably reduced until the resulting bottoms acquire a flash point approximating that of the stock which is to be used as a source of lubricating oil prepared by the normal or standard methods. These reduced bottoms are then added to a normal lubricating oil stock and the mixture reduced to the desired viscosity or flash, if necessary, treated with an acid, filtered and otherwise refined as desired.

35 We prefer to add the reduced residual bottoms to a lubricating oil stock which has been obtained during the distillation operation in which the lubricating oil stock is thrown over and condensed as a distillate. Such 40 lubricating oil distillates are encountered when it becomes necessary on an eastern or paraffine base stock to distill the stock over for the conversion of its amorphous wax content into wax of the crystalline state. 45 They are always encountered in separating the lubricating oil stocks from the tarry residue of asphaltic or mixed base crudes in the normal or standard methods of preparing lubricating oils from such asphaltic 50 or mixed base crudes.

As a variation from this preferred manner of carrying out our invention, we may first take the residual bottoms from the destructive distillation part of our process and 55 treat them with an acid after which they may be reduced to the desired viscosity and filtered or otherwise refined if desired, in order to make therefrom a finished high grade lubricating oil. This finished oil is

60 characterized by a rich green fluorescence. It is then mixed in desired proportions with a finished lubricating oil which has been prepared by the normal or standard methods, in which case there is imparted to the 65 resulting oil a rich green fluorescence.

We may also if desired distill the residual bottoms resulting from the destructive distillation part of our process and use the resulting distillate as a source for high grade lubricating oils as set forth in the copending 70 application referred to above and then mix the same in desired proportions with a finished lubricating oil stock which has been prepared by normal or standard methods.

By the practice of our invention we are 75 not only able to prepare an oil from an asphaltic base crude, and from a paraffine base overhead stock, possessing desired green fluorescence but we also produce an oil having certain other improved characteristics. For example, by destructively distilling a part of the stock from which our oil is made, to obtain the residuum which we employ, there is produced from this source 80 a certain portion of our finished oil which has been highly stabilized by the intense heat to which it has been subjected. Due to this intense heat marked chemical changes or molecular rearrangements have taken 85 place and certain unstable fractions, which would tend to break down if present in an oil used in internal combustion engines, are either cracked and distilled off or later removed from the residuum, or they are polymerized and retained in the oil in a much 90 more stable form. Such oils, in addition to possessing the rich green fluorescence are red in color when viewed by transmitted light. They are characterized by higher 95 Baumé viscosity-gravity ratio, i. e., for the same viscosity they are always found to be heavier than the lubricating oils prepared by the normal or standard practice.

It is also true that the lubricating oil 100 prepared from the residuum which we employ shows a marked reduction in the sulphur content. As a result, therefore, of blending this high grade stock with a lubricating stock which has been, or is to be, 105 treated for a lubricating oil in the normal manner, we impart to the latter a proportionate amount of these improved characteristics so that our final oil is of a character superior to oils made from the same crude by normal or standard methods. 110 These advantageous results are obtained whether a finished oil, prepared from the above described residuum, is blended with a finished oil prepared by normal methods or whether the residuum is first mixed after 115 being reduced to a required flash point, if desired, with the stock from which the finished oil is to be prepared, and the resulting mixture then treated for a final product.

We have also found that when the residuum resulting from the destructive distilling operation which we employ is added to the lubricating oil stock which is to be 120 treated in a normal or standard manner 125

there results, during the subsequent treatment of the mixture for a final product, a more rapid separation of the acid sludge resulting from the acid treatment of the stock. Furthermore, following the neutralizing step, we have found that the separation of the neutralized substances is more complete, so that the usual brightening operation is very much reduced and in some cases 10 obviated. Another and very important advantage of our invention is that petroleum oil can be treated, cracked or destructively distilled, and thereby a maximum production of gasoline obtained, simultaneously 15 with the production of the residuum which we employ as a source of our highly stabilized and green bloom producing stock.

Our invention is capable of numerous modifications and is not therefore limited 20 by the preceding description which has been given to illustrate our preferred process, but the invention is of the scope set forth in the following claims:

We claim:

- 25 1. The process of manufacturing a lubricating oil of green fluorescence from a petroleum oil normally yielding an oil of different fluorescence, which includes combining with such oil, oil from the residuum 30 of a cracking process wherein a petroleum oil has been subjected to the requisite temperature and pressure to decompose part of the oil into relatively lower boiling point oil and to stabilize the residuum.
- 35 2. A method of producing lubricating oil from petroleum oil, which includes subjecting petroleum oil to the requisite temperature and pressure to decompose a part of such oil to form relatively lower boiling point oil while stabilizing the residuum, and combining at least a part of such residuum with a petroleum oil containing a lubricating stock, and treating the resultant mixture to produce a finished lubricating oil.
- 40 3. The process of manufacturing lubricating oils having a green fluorescence, which includes combining a part of the residuum obtained from a cracking operation wherein the requisite temperature and pressure has been employed to decompose 45 part of the oil into relatively lower boiling point oil and to stabilize the residuum, with a lubricating stock of different fluorescence.
- 50 4. In the art of manufacturing lubricating oil from petroleum oil, combining with lubricating oil stock, part of the residuum of a cracking operation wherein petroleum oil is subjected to requisite temperature and 55 pressure to decompose part of the oil into relatively lower boiling point oil and to stabilize part of the oil and to produce materials imparting a green fluorescence to the residuum.
- 60 65 5. In the art of producing a lubricating

oil having a green fluorescence, that step in which oil from the residuum of a destructive distillation operation is combined with a lubricating oil stock prepared below the temperature and pressure at which any substantial part of the lubricating oil stock is 70 decomposed.

6. A method of producing lubricating oil, which includes subjecting petroleum oil to the requisite temperature and pressure to 75 decompose a part of such oil into relatively lower boiling point oil while substantially preventing vaporization of at least the relatively higher boiling point oil, so as to stabilize such undecomposed relatively high 80 boiling point oil, combining part of the stabilized oil with a lubricating oil stock separated from crude at a temperature and pressure below such decomposing and stabilizing conditions.

7. A method of producing lubricating oil which includes subjecting petroleum oil to the requisite temperature and pressure to decompose a part of such oil into relatively lower boiling point oil while substantially 90 preventing vaporization of at least the undecomposed relatively higher boiling point oil so as to stabilize such undecomposed relatively high boiling point oil, combining at least the lubricating oil stock from such stabilized oil with a petroleum lubricating oil stock separated from the crude by a normal process, that is one carried out at a temperature and pressure below such decomposing and stabilizing conditions, and refining together the combined stocks with sulphuric acid.

8. In the art of manufacturing lubricating oil from petroleum oil the combined operations including subjecting petroleum oil to the requisite temperature and pressure to decompose a part of the oil into relatively lower boiling point oil while substantially preventing vaporization of the undecomposed relatively higher boiling point oil, so as to stabilize such undecomposed relatively high boiling point oil, reducing such stabilized oil to separate therefrom a lubricating oil stock, mixing such stock with lubricating fractions obtained from petroleum oil by reducing or distillation operation carried out below such decomposing and stabilizing conditions of temperature and pressure, and treating the resultant mixture to finish the lubricating oil.

9. In the art of manufacturing lubricating oil from petroleum oil, the combined operations including subjecting petroleum oil to a stabilizing action carried out under a temperature not less than 650° F. and a pressure not less than 10 pounds per square inch, reducing the residuum to separate lubricating stock from the other constituents thereof, mixing such stock with lubricating oil stock separated from petroleum

oil below such stabilizing conditions, and refining the resultant mixture with sulfuric acid.

10. A lubricating oil possessing a green fluorescence comprising a combination of lubricating oil from the residue of a cracking process wherein the requisite temperature and pressure have been maintained to produce a polymerized and stabilized vis-

cous oil stock, and lubricating oil obtained from petroleum by operations carried out below such stabilizing conditions of temperature and pressure.

Signed at Richmond, Calif., this 17th day of April, 1924.

RICHARD W. HANNA.  
ORVILLE ELLSWORTH CUSHMAN.  
THEODORE WILLIAM DOELL.